# EUROPEAN PATENT APPLICATION

(11) **EP 4 671 398 A1**
(43) Date of publication of application: **31.12.2025**
(21) Application number: 23924173.0
(22) Date of filing: 07.11.2023
(51) Int. Cl.: C22C 38/00, C21D 7/04, C21D 9/46, C22C 38/60

(54) **STEEL SHEET AND MANUFACTURING METHOD THEREFOR**

(30) Priority: 22.02.2023 JP 2023026531; 22.02.2023 JP 2023026489; 22.02.2023 JP 2023026491
(71) Applicant: NIPPON STEEL CORPORATION, Chiyoda-ku Tokyo 100-8071 (JP)
(72) Inventor: MIYAKAWA, Taku, Tokyo 100-8071 (JP); YOKOYAMA, Takafumi, Tokyo 100-8071 (JP)
(74) Representative: Vossius & Partner Patentanwälte Rechtsanwälte mbB
(86) International application number: PCT/JP2023/040057
(87) International publication number: WO 2024/176529

(57) **Abstract**

The present invention provides a steel sheet having improved bendability after plastic working and excellent tensile strength, and also provides a manufacturing method therefor. A steel sheet according to the present invention is characterized by exhibiting a tensile strength of 1180 MPa or more, and having a prescribed chemical composition and steel structure, wherein the surface layer portion of the steel sheet has a deboronized layer where the luminescence intensities B30, B140, and B150 of B, as measured in the depth direction from the steel sheet surface by high-frequency glow discharge optical emission spectrometry, at the depth positions of 30 µm, 140 µm, and 150 µm from the steel sheet surface satisfy B30/B150<0.90 and 0.90≤B140/B150≤1.10, and in the surface layer portion of the steel sheet, the luminescence intensities C30, C140, and C150 of C, as measured in the depth direction from the steel sheet surface by high-frequency glow discharge optical emission spectrometry, at the depth positions of 30 µm, 140 µm, and 150 µm from the steel sheet surface satisfy C30/C150≤0.50 and 0.90≤C140/C150≤1.10.

## Description

### FIELD

The present invention relates to steel sheet and a method of production thereof.

### BACKGROUND

In recent years, improvement of the fuel economy of automobiles has been sought from the viewpoint of restrictions on emission of hothouse effect gases accompanying measures against global warming. High strength steel sheet is being increasingly used for lightening the weight of car bodies and securing safety in collision. In particular, recently, the need for ultra-high strength steel sheet with a tensile strength of 980 MPa or more has been rising.

Hot dip galvanized steel sheet used for automobile parts is being asked to be improved in not only strength, but also press formability, weldability, and various other aspects of workability required for forming parts. Specifically, excellent bendability is being sought from steel sheet from the viewpoint of press formability.

PTL 1 discloses steel sheet in which B is contained at the steel sheet surface layer part mainly in a precipitated state and inside of the steel sheet mainly in a solid solution state so as to improve the bendability.

PTL 2 discloses high strength steel sheet excellent in delayed fracture resistance of a cut end face and steel sheet base material having a martensite single phase structure, having a region with a KAM value (kernel average misorientation value) of a value of 1° or more comprising 50% or more of the total, and having a maximum tensile residual stress in the surface layer region down to the 1/4 depth position of sheet thickness from the surface of 80 MPa or less.

As art for the improvement of the bendability of high strength steel sheet, for example, PTL 3 describes high strength cold rolled steel sheet with a surface layer part mainly comprised of ferrite which is produced by decarburization of the steel sheet. Further, PTL 4 describes ultra-high strength cold rolled steel sheet having a soft layer at the surface layer part which is produced by annealing for decarburization of steel sheet.

### [CITATION LIST]

### [PATENT LITERATURE]

[PTL 1] WO2017/002883
[PTL 2] Japanese Unexamined Patent Publication No. 2015-155572
[PTL 3] Japanese Unexamined Patent Publication No. 10-130782
[PTL 4] Japanese Unexamined Patent Publication No. 5-195149

### SUMMARY

### [TECHNICAL FIELD]

Further, high strength steel sheet used for auto parts is being required to not break due to deformation by collision after being formed into a part. In particular, the steel sheet used for auto parts has to be excellent in not only bendability before press forming, but also bendability after plastic strain is introduced by press forming. In particular, keeping down the load drop due to fine cracks formed at the time of deformation by collision is sought from steel sheet for automobile use. However, improvement of the bendability after plastic strain is introduced has not necessarily been sufficiently studied up to now.

Therefore, the present invention has as its object the provision of steel sheet excellent in tensile strength and improved in bendability after plastic working and a method of production thereof.

### [SOLUTION TO PROBLEM]

The inventors engaged in repeated intensive studies for solving the above problem and as a result discovered that it is necessary to inhibit the formation and propagation of cracks after plastic working at the time of bending deformation for suppressing fracture in collision. Specifically, the inventors discovered that it is important to keep down the bending angle at the time of maximum load in a VDA bending test and a load drop after the maximum load. Further, the inventors discovered that it is possible to improve the bendability after plastic working by, as a means, forming a suitable deboronized layer at the surface layer part. The present invention was perfected based on these findings. The present invention includes the following aspects.

### (Aspect 1)

Steel sheet, in which steel sheet,
a chemical composition of the steel sheet contains, by mass%,
C: 0.06 to 0.30%,
Si: 0.01 to 2.50%,
Mn: 1.00 to 3.50%,
Ti: 0.001 to 0.100%,
B: 0.0005 to 0.0050%,
P: 0.050% or less,
S: 0.0100% or less,
Al: 1.500% or less,
N: 0.010% or less,
O: 0.0100% or less,
Cr: 0 to 1.00%,
Mo: 0 to 1.00%,
Cu: 0 to 1.00%,
Ni: 0 to 1.00%,
Co: 0 to 1.00%,
W: 0 to 1.00%,
Sn: 0 to 1.00%,
Sb: 0 to 0.50%,
Nb: 0 to 0.200%,
V: 0 to 1.00%,
As: 0 to 0.10%,
Zn: 0 to 1.00%,
Ca: 0 to 0.0100%,
Mg: 0 to 0.0100%,
Ce: 0 to 0.0150%,
Zr: 0 to 0.0100%,
La: 0 to 0.0150%,
Hf: 0 to 0.0100%,
Bi: 0 to 0.0100%,
an REM other than Ce and La: 0 to 0.0100%, and
bal.: Fe and impurities,
a steel structure in a range of a 1/8 depth position to 3/8 depth position of sheet thickness of the steel sheet comprises, by area%,
ferrite: 30% or less,
tempered martensite: 40% or more,
retained austenite: 8% or less,
fresh martensite: 10% or less,
total of pearlite and cementite: 5% or less, and
bal.: bainite,
a surface layer part of the steel sheet has a deboronized layer with an emission intensity of B, measured by high frequency glow discharge spectrometry in a depth direction from the steel sheet surface, satisfying the following formula (1) and formula (2),
further, a surface layer part of the steel sheet has an emission intensity of C, measured by high frequency glow discharge spectrometry in a depth direction from the steel sheet surface, satisfying the following formula (3) and formula (4), and
a tensile strength is 1180 MPa or more: $B 30 / B 150 < 0.90$ $0.90 \leq B 140 / B 150 \leq 1.10$ where,
   B30: emission intensity of B at depth position of 30 µm from the steel sheet surface
   B140: emission intensity of B at depth position of 140 µm from the steel sheet surface
   B 150: emission intensity of B at depth position of 150 µm from the steel sheet surface $C 30 / C 150 \leq 0.50$ $0.90 \leq C 140 / C 150 \leq 1.10$ where,
      C30: emission intensity of C at depth position of 30 µm from the steel sheet surface
      C140: emission intensity of C at depth position of 140 µm from the steel sheet surface
      C150: emission intensity of C at depth position of 150 µm from the steel sheet surface

### (Aspect 2)

The steel sheet according to the aspect 1, wherein the steel sheet surface has a hot dip galvanized layer or a hot dip galvannealed layer.

### (Aspect 3)

A method of production of steel sheet, which method of production of steel sheet comprising
a hot rolling step (a) of hot rolling a slab having a chemical composition comprising, by mass%,
C: 0.06 to 0.30%,
Si: 0.01 to 2.50%,
Mn: 1.00 to 3.50%,
Ti: 0.001 to 0.100%,
B: 0.0005 to 0.0050%,
P: 0.050% or less,
S: 0.0100% or less,
Al: 1.500% or less,
N: 0.010% or less,
O: 0.0100% or less,
Cr: 0 to 1.00%,
Mo: 0 to 1.00%,
Cu: 0 to 1.00%,
Ni: 0 to 1.00%,
Co: 0 to 1.00%,
W: 0 to 1.00%,
Sn: 0 to 1.00%,
Sb: 0 to 0.50%,
Nb: 0 to 0.200%,
V: 0 to 1.00%,
As: 0 to 0.10%,
Zn: 0 to 1.00%,
Ca: 0 to 0.0100%,
Mg: 0 to 0.0100%,
Ce: 0 to 0.0150%,
Zr: 0 to 0.0100%,
La: 0 to 0.0150%,
Hf: 0 to 0.0100%,
Bi: 0 to 0.0100%,
an REM other than Ce and La: 0 to 0.0100%, and
bal.: Fe and impurities at a 850 to 950°C finish rolling end temperature to obtain hot rolled steel sheet, then cooling the hot rolled steel sheet down to 450 to 650°C and coiling the hot rolled steel sheet,
a pickling step (b) of pickling the steel sheet obtained at the hot rolling step (a),
a cold rolling step (c) of cold rolling the steel sheet obtained by the pickling step (b) by a 30 to 75% rolling reduction to obtain a cold rolled steel sheet,
a heat treatment step (d) of heat treating the steel sheet obtained at the cold rolling step (c), and
a grinding step (e), before or after the pickling step (b), of using a rotary type grinding brush containing an abrasive to grind the front and back surfaces of the steel sheet obtained at the hot rolling step (a) or the steel sheet obtained at the pickling step (b),
in the hot rolling step (a), finish rolling comprises three passes or more, the rolling reduction of the respective passes of the final three passes of the finish rolling is 20% or more, the time between passes is within 1 second, the entry side steel sheet temperature before the final three passes is 1000°C or less, and the time from the completion of the final pass to the start of cooling is within 3 seconds,
in the grinding step (e), a rotational speed R (rpm) of the grinding brush, a diameter D (m) of the grinding brush, and a running speed V (m/min) of the steel sheet satisfy the following formula (5),
the heat treatment step (d) further provided with
a step (d-1) of heating the steel sheet obtained at the cold rolling step (c) from 650°C to a maximum heating temperature of the Ac1+50°C or more and 950°C or less by an average heating speed of 0.5 to 500°C/s,
a step (d-2) of holding the steel sheet obtained at the cold rolling step (c) at the maximum heating temperature for 1 second to 300 seconds,
a step (d-3) of cooling the steel sheet obtained at the cold rolling step (c) down to the Ms point-100°C or less, at which step, cooling from 700°C to 500°C by a 10°C/s or more average cooling speed, and
a step (d-4) of holding the steel sheet obtained at the cold rolling step (c) at 200 to 350°C for 1 to 600 seconds,
at step (d-1), the atmosphere in the surroundings of the steel sheet obtained at the cold rolling step (c) having a steam partial pressure pH₂O and hydrogen partial pressure pH₂ satisfying the following formula (6): $\begin{matrix}\frac{R ⋅ D}{V} > 10 \left(5\right) \\ - 1.0 \leq log \left({pH}_{2}{O / pH}_{2}\right) \leq - 0.1 \left(6\right)\end{matrix}$

### (Aspect 4)

The method of production of steel sheet according to the aspect 3, wherein
the hot rolling step (a) further comprises a step of retaining the heat of the hot rolled steel sheet after coiling within 30 minutes in a heat insulating vessel with inside walls covered by a heat insulating material, wherein
a peak temperature of an atmospheric temperature inside of the heat insulating vessel is 500 to 650°C, and the time from the atmospheric temperature to the peak temperature is 1 to 8 hours.

### [ADVANTAGEOUS EFFECTS OF INVENTION]

According to the present invention, it is possible to obtain steel sheet excellent in tensile strength and excellent in bendability after plastic working.

### BRIEF DESCRIPTION OF DRAWINGS

FIG. 1 is a view schematically showing a cross-section of a plated steel sheet 1 including a base steel sheet 2 according to one embodiment of the present invention sliced in the sheet thickness direction.

### DESCRIPTION OF EMBODIMENTS

Below, a plated steel sheet including a steel sheet of one embodiment of the present invention as a base steel sheet will be explained in detail while referring to FIG. 1. It should be noted that, FIG. 1 is a view schematically showing a cross-section of a plated steel sheet 1 including a base steel sheet 2 according to one embodiment of the present invention sliced in the sheet thickness direction.

The present invention prescribes the features of a specific position of the steel sheet in the sheet thickness direction. In the following explanation, these features will sometimes be explained using a position of the steel sheet in the sheet thickness direction based on the steel sheet surface.

It should be noted that, the "sheet thickness direction" and the "depth direction" of the steel sheet are synonymous, and therefore in this Description, a position of the steel sheet in the sheet thickness direction based on the steel sheet surface will sometimes be called the "depth position".

In relation to this, in this Description, the "x/y depth position of sheet thickness (in this case, 'x' and 'y' are natural numbers satisfying x<y)" means the position in the sheet thickness direction of the steel sheet from the surface, i.e., the steel sheet surface, in the sheet thickness direction toward the center part of the steel sheet by exactly the distance of x/y of the sheet thickness (depth). For example, if the sheet thickness of the steel sheet was "t" mm, the "1/8 depth position of the sheet thickness" means the position becoming the depth of 1t/8 mm in the sheet thickness direction from the steel sheet surface.

In this case, regarding the "steel sheet surface" based on the position of the sheet thickness direction of the steel sheet, i.e., the depth position of the steel sheet, in this Description, in the later explained high frequency glow discharge spectrometry (below, sometimes referred to as "high frequency GDS analysis"), the depth position where the emission intensity of Fe reaches 0.7 time the inside emission intensity of Fe is defined as the 0 µm position and this 0 µm position is deemed the steel sheet surface. The "inside emission intensity of Fe" is the emission intensity of Fe at a region of a sufficient depth of the base steel sheet. This region is a region with almost no change in concentration of Fe in the depth direction and a region judged as "steel" as technical common sense. The inside emission intensity of Fe, for example, may be made the emission intensity of Fe at a sputter time of 1000 seconds.

It should be noted that, the "steel sheet" covered by the present invention is sometimes the "base steel sheet" having some sort of covering on its surface such as the plated steel sheet 1 shown in FIG. 1. In such a case, the "steel sheet surface" forming the basis for the depth position of the steel sheet becoming the steel sheet surface of the base steel sheet, but in the same way as the above, the emission intensity of Fe at the high frequency GDS analysis is the depth position reaching 0.7 time of the inside emission intensity of Fe, i.e., the 0 µm position.

For example, in the plated steel sheet 1 shown in FIG. 1, the steel sheet surface is the position of the symbol "S_{d}" shown by the broken lines near the interface of the base steel sheet 2 and the plating layer 3. This position, as explained above, is the depth position where the emission intensity of Fe reaches 0.7 time the inside emission intensity of Fe in high frequency GDS analysis, i.e., the 0 µm position.

Further, the expression of "depth position of 30 µm from the steel sheet surface" etc. also similarly means the position moved in the sheet thickness direction from the steel sheet surface by exactly the distance of 30 µm toward the center part of the steel sheet. For example, in the plated steel sheet 1 shown in FIG. 1, the depth position P₃₀ of 30 µm from the steel sheet surface S_{d} is the position moved in the sheet thickness direction from the steel sheet surface S_{d} by exactly the distance of 30 µm toward the center part of the steel sheet.

### <Plated Steel Sheet>

As shown in FIG. 1, the plated steel sheet 1 is plated steel sheet having the base steel sheet 2 of the present embodiment and a plating layer 3 provided on both surfaces of the base steel sheet 2. It should be noted that, the plating layer 3 may also be provided on one surface of the base steel sheet 2.

Further, the plated steel sheet 1, as shown in FIG. 1, has a surface layer part P_{S} defined as a region in the sheet thickness direction to a depth position P₁₅₀ from the steel sheet surface S_{d} of 150 µm.

### <Base Steel Sheet>

Further, in the present embodiment, the base steel sheet 2 has the following features:
First, the chemical composition of the base steel sheet 2 contains, by mass%,
C: 0.06 to 0.30%,
Si: 0.01 to 2.50%,
Mn: 1.00 to 3.50%,
Ti: 0.001 to 0.100%,
B: 0.0005 to 0.0050%,
P: 0.050% or less,
S: 0.0100% or less,
Al: 1.500% or less,
N: 0.010% or less,
O: 0.0100% or less,
Cr: 0 to 1.00%,
Mo: 0 to 1.00%,
Cu: 0 to 1.00%,
Ni: 0 to 1.00%,
Co: 0 to 1.00%,
W: 0 to 1.00%,
Sn: 0 to 1.00%,
Sb: 0 to 0.50%,
Nb: 0 to 0.200%,
V: 0 to 1.00%,
As: 0 to 0.10%,
Zn: 0 to 1.00%,
Ca: 0 to 0.0100%,
Mg: 0 to 0.0100%,
Ce: 0 to 0.0150%,
Zr: 0 to 0.0100%,
La: 0 to 0.0150%,
Hf: 0 to 0.0100%,
Bi: 0 to 0.0100%,
an REM other than Ce and La: 0 to 0.0100%, and
bal.: Fe and impurities.

The steel structure in the range of the 1/8 depth position to the 3/8 depth position of sheet thickness of the base steel sheet 2 comprises, by area%, ferrite: 30% or less, tempered martensite: 40% or more, retained austenite: 8% or less, fresh martensite: 10% or less, total of pearlite and cementite: 5% or less, and bal.: bainite.

Further, the surface layer part P_{S} of the base steel sheet 2 has a deboronized layer P_{B} with an emission intensity of B, measured by high frequency glow discharge spectrometry in the depth direction from the steel sheet surface S_{d}, satisfying the following formula (1) and formula (2): $B 30 / B 150 < 0.90$ $0.90 \leq B 140 / B 150 \leq 1.10$ where,
B30: emission intensity of B at depth position of 30 µm from steel sheet surface S_{d}
B 140: emission intensity of B at depth position of 140 µm from steel sheet surface S_{d}
B150: emission intensity of B at depth position of 150 µm from steel sheet surface S_{d}

Further, the surface layer part P_{S} of the base steel sheet 2 satisfies an emission intensity of C, measured by high frequency glow discharge spectrometry from the steel sheet surface S_{d} in the depth direction, satisfying the following formula (3) and formula (4): $C 30 / C 150 \leq 0.50$ $0.90 \leq C 140 / C 150 \leq 1.10$ where,
C30: emission intensity of C at depth position of 30 µm from steel sheet surface S_{d}
C140: emission intensity of C at depth position of 140 µm from steel sheet surface S_{d}
C150: emission intensity of C at depth position of 150 µm from steel sheet surface S_{d}

Further, the tensile strength of the base steel sheet 2 is 1180 MPa or more.

Below, these features in the base steel sheet 2 will be explained in detail.

### (Chemical Composition)

First, the reasons for limiting the chemical composition of the base steel sheet according to the present invention (below, sometimes simply referred to as the "steel sheet") in the above-mentioned way will be explained. It should be noted that, in this Description, the "%"s prescribing the chemical composition, unless particularly indicated otherwise, are all "mass%". Further, in this Description, the "to" indicating a numerical range, unless particularly indicated otherwise, is used in the sense including the numbers described before and after it as the lower limit value and upper limit value.

### (C: 0.06 to 0.30%)

C (carbon) is an element essential for securing the strength of steel sheet. From the viewpoint of obtain the required high strength, the C content is 0.06% or more. The C content may be 0.07% or more, 0.08% or more, or 0.10% or more. Further, from the viewpoint of workability and weldability, the C content is 0.30% or less. The C content may be 0.29% or less, 0.28% or less, or 0.25% or less.

### (Si: 0.01 to 2.50%)

Si (silicon) is an element suppressing the formation of iron carbides and contributing to improvement of the strength and shapeability. From the viewpoint of the strength, shapeability, and weldability, the Si content is 0.01 to 2.50%. The Si content may also be 0.05% or more, 0.10% or more, 0.15% or more, or 0.20% or more. Further, the Si content may also be 2.20% or less, 2.00% or less, or 1.90% or less.

### (Mn: 1.00 to 3.50%)

Mn (manganese) is a powerful austenite stabilizing element and an element effective for raising the strength of steel sheet. From the viewpoint of strength, weldability, and low temperature toughness, the content of Mn is 1.00 to 3.50%. The Mn content may be 1.10% or more, 1.30% or more, or 1.50% or more. Further, the Mn content may also be 3.30% or less, 3.10% or less, or 3.00% or less.

### (Ti: 0.001 to 0.100%)

Ti (titanium) is an element effective for raising the strength of steel sheet. From the viewpoints of raising the strength and cost, the Ti content is 0.001 to 0.100%. The Ti content may also be 0.005% or more, 0.010% or more, 0.015% or more, or 0.020% or more. Further, the Ti content may also be 0.080% or less, 0.070% or less, or 0.050% or less.

### (B: 0.0005 to 0.0050%)

B (boron) is an element raising the quenchability of steel sheet and raising the strength. It is an essential element in the present invention. In the present invention, by forming the later explained deboronized layer at the surface layer part of the steel sheet, it is possible to improve the bendability after plastic working the steel sheet. From the viewpoint of forming a suitable deboronized layer, the B content is 0.0005 to 0.0050%. The B content may also be 0.0007% or more, 0.0010% or more, or 0.0015% or more. Further, the B content may also be 0.0040% or less, 0.0035% or less, or 0.0030% or less.

### (P: 0.050% or Less)

P (phosphorus) is an element contained in steel as an impurity. It contributes to higher strength of the steel sheet as well by solution strengthening, but from the viewpoints of weldability and toughness, the P content is 0.050% or less. The P content is preferably 0.045% or less, 0.035% or less, or 0.020% or less. P is not an essential element. The lower limit of the P content is 0%. However, to greatly reduce the P content, the dephosphorization cost becomes higher, therefore from the viewpoint of economy, the lower limit of the P content may be 0.0001%, 0.0005%, or 0.001%.

### (S: 0.0100% or Less)

S (sulfur) is an element contained in steel as an impurity and an element forming MnS in steel sheet to cause deterioration of the toughness and hole expandability. Therefore, from the viewpoint of suppressing the deterioration of the toughness and hole expandability, the S content is 0.0100% or less. The S content is preferably 0.0050% or less, 0.0040% or less, or 0.0030% or less. S is not an essential element. The lower limit of the S content is 0%. However, to greatly reduce the S content, the desulfurization cost becomes higher, so from the viewpoint of economy, the lower limit of the S content may be 0.00001%, 0.00005%, or 0.0001%.

### (Al: 1.500% or Less)

Al (aluminum) is an element contained for deoxidation of steel and an element not required to be contained in the final product steel sheet. Therefore, the lower limit of the Al content is 0%. However, to obtain a sufficient effect of deoxidation, the final product steel sheet may have Al added to it at the time of deoxidation so that Al is contained in 0.0001% or more, 0.0005% or more, or 0.001% or more. From the viewpoint of the load at the time of hot rolling due to making the transformation temperature of the steel rise, the upper limit of the Al content is 1.500%. The Al content is preferably 1.200% or less, 1.000% or less, or 0.800% or less.

### (N: 0.010% or Less)

N (nitrogen) is an element contained in steel as an impurity and an element which, when its content is more than 0.010%, forms rough nitrides in the steel and causes the bendability and hole expandability to deteriorate. Therefore, the N content is 0.010% or less. The N content is preferably 0.008% or less, 0.006% or less, or 0.005% or less. N is not an essential element, therefore the lower limit of the N content is 0%. However, to greatly reduce the N content, the denitridation cost becomes high, therefore from the viewpoint of economy, the lower limit of the N content may also be 0.0001%, 0.0005%, or 0.001%.

### (O: 0.0100% or Less)

O (oxygen) is an element contained in steel as an impurity and an element, which if its content is more than 0.0100%, forms coarse oxides in the steel to cause deterioration of the bendability and hole expandability. Therefore, the O content is 0.0100% or less. The O content is preferably 0.0080% or less, 0.0060% or less, or 0.0050% or less. O is not an essential element, therefore the lower limit of the O content is 0%. However, from the viewpoint of the production cost, the lower limit of the O content may also be 0.00001%, 0.00005%, or 0.0001%.

The basic chemical composition of the base steel sheet 2 in the present embodiment is as explained above. Further, the base steel sheet 2 may also contain any of the following optional elements in accordance with need.

### (Cr: 0 to 1.00%, Mo: 0 to 1.00%, Cu: 0 to 1.00%, Ni: 0 to 1.00%, Co: 0 to 1.00%, W: 0 to 1.00%, Sn: 0 to 1.00%, Sb: 0 to 0.50%, Nb: 0 to 0.200%, V: 0 to 1.00%, As: 0 to 0.10%, and Zn: 0 to 1.00%)

Cr (chromium), Mo (molybdenum), Cu (copper), Ni (nickel), Co (cobalt), W (tungsten), Sn (tin), Sb (antimony), Nb (niobium), V (vanadium), As (arsenic), and Zn (zinc) are all elements effective for raising the strength of steel sheet. For this reason, one or more of these elements may be added in accordance with need. From the viewpoint of the effect and cost due to inclusion of these elements, the contents of these elements are Cr: 0 to 1.00%, Mo: 0 to 1.00%, Cu: 0 to 1.00%, Ni: 0 to 1.00%, Co: 0 to 1.00%, W: 0 to 1.00%, Sn: 0 to 1.00%, Sb: 0 to 0.50%, Nb: 0 to 0.200%, V: 0 to 1.00%, As: 0 to 0.10%, and Zn: 0 to 1.00%. The contents of these elements may also be 0.005% or more or 0.010% or more.

### (Ca: 0 to 0.0100%, Mg: 0 to 0.0100%, Ce: 0 to 0.0150%, Zr: 0 to 0.0100%, La: 0 to 0.0150%, Hf: 0 to 0.0100%, Bi: 0 to 0.0100%, and REM Other Than Ce and La: 0 to 0.0100%)

Ca (calcium), Mg (magnesium), Ce (cerium), Zr (zirconium), La (lanthanum), Hf (hafnium), and an REM other than Ce and La (rare earth metals) are all elements contributing to fine dispersion of inclusions in the steel. Bi (bismuth) is an element mitigating microsegregation of Mn, Si, and other substitution type alloy elements in the steel. These elements contribute to improvement of the workability of steel sheet, so, in accordance with need, one or more of these elements may be added. From the viewpoint of the workability and ductility, the upper limits of the contents of Ca, Mg, Zr, Hf, Bi, and REMs other than Ce and La are respectively 0.0100%, while the upper limits of the contents of Ce and La are respectively 0.0150%. The contents of these elements may also respectively be 0.0005% or more or 0.0010% or more.

In the present embodiment, the balance besides the above elements of the base steel sheet 2 is comprised of Fe and impurities. In this case, the "impurities" contained in the balance besides the above constituents are constituents entering due to the ore, scrap, or other raw materials and other various factors in the production process when industrially producing the steel sheet. The impurities include constituents not intentionally added to the base steel sheet 2. Further, the impurities contained in the balance are elements other than the constituents explained above and also include elements contained in steel sheet within an extent where the actions and effects distinctive to the elements in the impurities do not affect the properties of the base steel sheet 2.

It should be noted that if the steel sheet is surface treated steel sheet, the chemical composition is the contents of the base steel sheet from which the covering at the surface has been peeled off. Further, in the case where the steel sheet is steel sheet not accompanied by a plating layer or a surface treated layer or other covering, the chemical composition is the content of the steel sheet itself.

The chemical composition of the steel sheet may be measured by a general analysis method. For example, the chemical composition of the steel sheet may be measured by using inductively coupled plasma-atomic emission spectrometry (ICP-AES). Specifically, for example, the front and back of the steel sheet are ground down to depth positions of 200 µm from the steel sheet surfaces to obtain a test piece. An ICPS-8100 or other measuring device made by Shimadzu Corporation can be used under conditions based on calibration curves prepared in advance to thereby identify the chemical composition of the steel sheet. C and S, which cannot be measured by ICP-AES, can be measured using the combustion-infrared absorption method, N can be measured using the inert gas melting-thermal conductivity method, and O can be measured using the inert gas melting-nondispersive type infrared absorption method.

### [Steel Structure Inside of Steel Sheet]

Next, the reasons for limitation of the internal structure of the base steel sheet 2 according to the present embodiment will be explained. It should be noted that, in this Description, the "%" prescribing the steel structure all mean "area%" unless particularly indicated otherwise.

### (Ferrite: 30% or Less)

Ferrite is excellent in ductility, but is a soft structure. To improve the elongation of steel sheet, it may be included in accordance with the required strength and ductility. From the viewpoint of the balance of strength and ductility, the upper limit of the ferrite content is 30%. The ferrite content may be 25% or less or 20% or less. The ferrite content may also be 0% and may also be 3% or more, 5% or more, or 10% or more.

### (Tempered Martensite: 40% or More)

Tempered martensite is a high strength and tough structure and is also a structure raising the tensile strength and bending load of steel sheet. To obtain the desired tensile strength and bendability, the lower limit of the tempered martensite content is 40% or more. The tempered martensite content is preferably 50% or more, 60% or more, 70% or more, or 80% or more.

### (Retained Austenite: 8% or Less)

Retained austenite is a structure contributing to improvement of the ductility of steel sheet by the effect of work induced transformation. On the other hand, retained austenite transforms induced by work by prestrain and transforms to martensite as quenched, therefore sometimes causes deterioration of the bendability of steel sheet. If the retained austenite content is more than 8%, the load drop after the VDA bending load drop becomes remarkable. Therefore, the retained austenite content is 8% or less. The retained austenite content is preferably 6% or less, 5% or less, or 4% or less. It should be noted that the retained austenite content may also be 0% or more, 1% or more, or 2% or more.

### (Fresh Martensite: 10% or Less)

Fresh martensite is also a high strength structure and a structure raising the tensile strength and bending load. On the other hand, fresh martensite is a brittle structure, and therefore if, in particular, the fresh martensite content is more than 10% it becomes starting points of fracture at the time of plastic deformation and local ductility of the steel sheet is sometimes made to deteriorate. Therefore, the fresh martensite content is 10% or less. The fresh martensite content is preferably 8% or less, 7% or less, or 5% or less. The fresh martensite content may also be 0% or more, 1% or more, 2% or more, or 3% or more.

### (Total of Pearlite and Cementite: 5% or Less)

Pearlite contains hard and coarse cementite and becomes starting points of fracture at the time of plastic deformation, and therefore if, in particular, the total content of the pearlite and cementite is more than 5%, sometimes the local ductility of the steel sheet is made to deteriorate. Therefore, the total content of the pearlite and cementite is 5% or less. The total content of pearlite and cementite may be 3% or less or 2% or less. In this case, "cementite" covers coarse particles of a circle equivalent diameter of more than 1 µm. "Fine cementite" precipitating in bainite or martensite is not included.

The balance structure other than the above structures may also be 0%, but if there is such a balance structure present, that balance structure is bainite. Furthermore, the bainite of the balance structure may be either of upper bainite and lower bainite and may be mixed structures of the same.

The steel structure fractions are evaluated by the SEM-EBSD method (electron backscattered diffraction method) and SEM secondary electron image observation.

First, a sample is taken from the steel sheet using a cross-section of sheet thickness parallel to the rolling direction as an examined surface, the examined surface is machine ground to finish it to a mirror surface, then the surface is electrolytically polished. Next, in one or more examined fields in the range at the 1/8 depth position to 3/8 depth position of sheet thickness of the steel sheet at the examined surface, a region of a total of 2.0×10⁻⁹m² or more in area is analyzed for crystal structure and orientation by the SEM-EBSD method. For analysis of the data obtained by the EBSD method, "OIM Analysys (TM) 6.0" made by TSL is used. Further, the distance between evaluation points (step) is 0.10 µm. The region judged to be FCC iron from the results of observation is deemed retained austenite. Furthermore, a crystal grain boundary map having boundaries with a crystal orientation difference of 15 degrees or more as grain boundaries is obtained.

Next, the same sample as the one examined by EBSD is corroded by Nital. This sample is examined by secondary electron images at the same fields as the EBSD measurement. To examine the same fields as at the time of EBSD measurement, a Vickers indentation or other mark may also be made in advance. From the obtained secondary electron images, the area ratios of the ferrite, retained austenite, bainite, tempered martensite, fresh martensite, and pearlite are measured.

Regions having substructures in the grains and having several variants of cementite, more specifically two or more types of variants, are judged to be tempered martensite. Regions having cementite precipitated in a lamellar form are judged to be pearlite. In the fields including various substructures, regions with relatively small brightness and no substructures observed are judged to be ferrite. Regions with large brightnesses and with substructures not appearing by etching are judged to be fresh martensite and retained austenite. The area ratios of the different structures are calculated by the point counting method to obtain the area ratios of the structures. The finer the grid spacing when point counting, the more accurate the values obtained. The grid spacing, for example, may be made a 2 µm spacing.

If the area ratio of the total of the structures obtained by the above method of evaluation is less than 100%, the balance regions are judged as bainite. Further, if the area ratio of the total of the structures obtained by the above method of evaluation is more than 100%, the value obtained by multiplying the area ratio of the structures by 100/(area ratio of total of structures) is made the area ratio of the structures.

### [Deboronized Layer]

In the present embodiment, the base steel sheet 2, as explained above, has a deboronized layer P_{B} at the surface layer part P_{S}. In this Description, a portion where the emission intensity of B, measured by high frequency glow discharge spectrometry (high frequency GDS analysis) in the depth direction from the steel sheet surface, satisfies the following formula (1) and formula (2) is defined as the "deboronized layer".
$B 30 / B 150 < 0.90$ $0.90 \leq B 140 / B 150 \leq 1.10$

In this case, B30, B140, and B150 are respectively, when measured by high frequency GDS analysis from the steel sheet surface in the sheet thickness direction, the emission intensity of B at a depth position of 30 µm from the steel sheet surface, the emission intensity of B at a depth position of 140 µm from the steel sheet surface, and the emission intensity of B at a depth position of 150 µm from the steel sheet surface.

The measurement by high frequency GDS analysis is performed at any five positions. B30, B140, and B150 are respectively the average values of emission intensity of B at depth positions of 30 µm, 140 µm, and 150 µm from the steel sheet surface at the any five positions. The measurement conditions are as follows:

B30, B140, and B150 are respectively measured using a high frequency glow discharge spectrometer. Specifically, the method is used of making the surface of the steel sheet to be measured an Ar atmosphere, applying voltage to generate glow plasma, and in that state causing sputtering at the surface of the steel sheet while analyzing the sheet in the depth direction. Further, the emission spectral wavelengths distinctive to the elements emitted due to excitation of atoms in the glow plasma are used to identify the elements contained in the steel sheet and estimate the emission intensities of the identified elements.

The depth direction data can be estimated from the sputter time. Specifically, by using standard samples in advance to find the relationship of the sputter time and sputter depth, it is possible to convert the sputter time to the sputter depth. Therefore, the sputter depth converted from the sputter time can be defined as the depth from the steel sheet surface. The sputter time is set so that at least the sputter depth exceeds 150 µm.

In the high frequency GDS analysis, a commercially available analysis apparatus can be used. In the present embodiment, a high frequency glow discharge spectrometer GD-Profiler2 (TM) made by Horiba is used. The detection pitch is 0.1 second. The obtained data is stripped of the background, then filtered. The filtering is performed by the moving average method. Specifically, the moving average of a total of 51 points of the center point+front/back 25 points is found. The values of the times corresponding to the 30 µm depth, 140 µm depth, and 150 µm depth are respectively B40, B140, and B150. The other measurement conditions are as follows:
Ar gas pressure: 600 Pa
Anode diameter: 4 mmφ
RF output: 35W

It should be noted that, in this Description, as explained above, the depth position where the emission intensity of Fe according to high frequency GDS analysis reaches 0.7 time the inside emission intensity of Fe is defined as the 0 µm position, but the inside emission intensity of Fe in this definition may, for example, be made the emission intensity of Fe at the sputter time of 1000 seconds.

The above formula (1) means the boron concentration at the depth position of 30 µm from the steel sheet surface is less than 0.90 time the boron concentration at the depth position of 150 µm. By satisfying this formula (1), when the steel sheet is plastically worked, the metallostructure near the steel sheet surface becomes harder to be damaged.

In formula (1), B30/B150 may be 0.80 or less, less than 0.80, 0.70 or less, less than 0.70, 0.60 or less, or less than 0.60. Further, B30/B150 may also be 0, but may also be 0.10 or more, 0.20 or more, or 0.30 or more.

Formula (2) means the emission intensity of B at the depth position of 140 µm from the steel sheet surface and the Be emission intensity at the depth position of 150 µm from the steel sheet surface are roughly equal. In other words, the region where the deboronized layer P_{B} can be formed in the present embodiment means down to the depth position of 150 µm from the steel sheet surface. By satisfying this formula (2), it is possible to prevent the depth position of 150 µm or more from the steel sheet surface from excessively ending up softening and secure the steel sheet strength.

By forming the above such deboronized layer P_{B}, it is possible to improve the bendability after plastic working. The reason why such an effect is obtained is not clear, but there may be a possibility of the damage to the metallostructure (for example, formation of microvoids etc.) when receiving plastic working being slighter in the soft layer of the surface layer formed by the deboronized layer P_{B} compared with the soft layer of the surface layer formed by the decarburized layer.

Further, in addition to the above deboronized layer P_{B}, to suppress progression of cracks after formation of cracks, the surface layer part P_{S} of the base steel sheet 2 has to be decarburized (below, sometimes simply referred to as "decarburization"). Specifically, at the surface layer part P_{S} of the base steel sheet 2, the emission intensity of C, measured by high frequency glow discharge spectrometry (high frequency GDS analysis) in the depth direction from the steel sheet surface, satisfies the following formula (3) and formula (4).
$C 30 / C 150 \leq 0.50$ $0.90 \leq C 140 / C 150 \leq 1.10$

In this case, C30, C140, and C150 are respectively, when measured from the steel sheet surface in the sheet thickness direction by high frequency GDS analysis, the emission intensity of C at the depth position of 30 µm from the steel sheet surface, the emission intensity of C at the depth position of 140 µm from the steel sheet surface, and the emission intensity of C at the depth position of 150 µm from the steel sheet surface.

The measurement by high frequency GDS analysis is performed at any five positions. C30, C140, and C150 are respectively the average values of the emission intensity of C at depth positions of 30 µm, 140 µm, and 150 µm from the steel sheet surface at the any five positions. The measurement conditions are similar to the above-mentioned B30, B140, and B150.

The above formula (3) means that the carbon concentration of the depth position of 30 µm from the steel sheet surface is 0.50 time or less of the carbon concentration at the depth position of 150 µm and that decarburization proceeds up to the depth position of 30 µm. By decarburization so as to satisfy the formula (3), when the steel sheet is plastically worked, the metallostructure at the deboronized layer becomes harder to be damaged and progression of cracks after formation of cracks can be easily suppressed.

In the above formula (3), C30/C150 may be 0.45 or less, 0.40 or less, or 0.35 or less. Further, C30/C150 may also be 0, but may also be 0.10 or more, 0.15 or more, or 0.20 or more.

The degree of the decarburization can be controlled by adjusting the atmosphere up to heating to the maximum heating temperature at the heat treatment of the method of production of the steel sheet explained later.

The formula (4) means that the emission intensity of C at the depth position of 140 µm from the steel sheet surface and the emission intensity of C at the depth position of 150 µm from the steel sheet surface are roughly equal. It should be noted that the C concentration at the depth position of 150 µm from the steel sheet surface becomes roughly equal to the C concentration at the center of sheet thickness of the steel sheet surface. By satisfying this formula (4), it is possible to prevent the depth position of 150 µm or more from the steel sheet surface from ending up excessively softening and secure the steel sheet strength.

### [Tensile Strength: 1180 MPa or More]

In the present embodiment, the tensile strength of the base steel sheet 2 is 1180 MPa or more. The base steel sheet 2 of the present embodiment, even if the tensile strength is such a high strength, has the above-mentioned decarburized deboronized layer P_{B}, therefore is excellent in bendability after plastic working. The tensile strength of the base steel sheet 2 may also be 1200 MPa or more, 1300 MPa or more, 1400 MPa or more, or 1500 MPa or more. It should be noted that the upper limit of the tensile strength of the base steel sheet 2 is not particularly limited, but from the viewpoint of the toughness and shapeability, for example, it may be 4000 MPa or less, 3000 MPa or less, or 2000 MPa or less.

It should be noted that the tensile strength (TS) of the steel sheet can be measured in the following way. First, a No. 5 test piece of JIS Z 2241: 2011 having a direction perpendicular to the rolling direction as a longitudinal direction is taken from the center part of width of the steel sheet to be measured. Next, this test piece can be used for performing a tensile test based on JIS Z 2241: 2011 to measure the tensile strength TS (MPa).

Further, if obtaining a test piece from the steel sheet to be measured is difficult, it is possible to measure the Vickers hardness of the steel sheet and use the measured value of the Vickers hardness to derive the tensile strength from the following correlation formula (Correlation Between Static Strength Parameters, Fumihiko Hasegawa, Junichi Arai, Tsuneshichi Tanaka, "Materials", Vol. 39, No. 442, P. 859 to 863).$Hv = 0.301 \times TS + 5.701$ where, in the above formula, "Hv" indicates the Vickers hardness and "TS" indicates the tensile strength (MPa).

The Vickers hardness of the steel sheet can be measured in accordance with JIS Z 2244: 2009. Specifically, the Vickers hardness of the steel sheet can be obtained by performing measurement by a load of 1 kgf (about 9.80N) 10 times at a 1/4 depth position of the sheet thickness of the steel sheet and finding the average value of the 10 measured values. At this time, the interval between the measurement positions is made a distance of 3X or more of the indentations.

### [Plating Layer]

As explained above, in the present embodiment, both sides of the base steel sheet 2 have the plating layer 3. The plating layer 3 may also be a hot dip galvanized layer or hot dip galvannealed layer having any known composition. The plating layer 3 may also include Al and other added elements besides Zn. Further, the amount of deposition of the plating layer 3 is not particularly limited and may be a general amount of deposition.

It should be noted that the plating layer 3 may be provided at only one surface of the base steel sheet 2 and may be provided at any surface of the base steel sheet 2. In the steel sheet of the present invention, it is not essential that the surface of the steel sheet have a plating layer.

### (Thickness of Steel Sheet)

The thickness of the steel sheet of the present invention is not particularly limited. For example, it may be made a thickness similar to the steel sheet used for automobile parts. As such a thickness of the steel sheet, for example, a 0.5 to 3.0 mm thickness may be mentioned. The thickness of the steel sheet may also be 0.7 mm or more, 0.8 mm or more, or 1.0 mm or more. Further, the thickness of the steel sheet may also be 2.8 mm or less, 2.5 mm or less, or 2.0 mm or less.

### <Method of Production of Steel Sheet>

Next, the method of production of steel sheet according to one embodiment of the present invention will be explained. The following explanation is intended to illustrate the characteristic method for production of the steel sheet according to an embodiment of the present invention and is not intended to limit the steel sheet to one produced by the method of production explained below.

The method of production of the steel sheet includes a hot rolling step (a) of hot rolling a slab having a specific chemical composition to obtain a hot rolled steel sheet (below, sometimes simply referred to as "step (a)"), a grinding step (e) of grinding the hot rolled steel sheet by a rotary grinding brush (below, sometimes simply referred to as "step (e)"), a pickling step (b) of pickling after grinding (below, sometimes simply referred to as "step (b)"), a cold rolling step (c) of cold rolling the pickled hot rolled steel sheet to obtain cold rolled steel sheet (below, sometimes simply referred to as "step (c)"), and a heat treatment step (d) of heat treating the cold rolled steel sheet (below, sometimes simply referred to as "step (d)".

Below, preferable conditions etc. of these steps will be explained in detail.

### [Hot Rolling Step (a)]

First, a slab having the following specific chemical composition is hot rolled under predetermined conditions to obtain a hot rolled steel sheet, then the hot rolled steel sheet is cooled down to a predetermined temperature and coiled in a hot rolling step (a). In the hot rolling step, a slab having the following specific chemical composition is heated before hot rolling.

In this case, regarding the chemical composition of the slab, if analyzing the chemical composition of the finally obtained steel sheet by the above-mentioned method of analysis, it can be confirmed that there is substantially no difference from the chemical composition of the slab.

Therefore, the chemical composition of the slab basically is the same as the above-mentioned chemical composition of the steel sheet. In other words, the chemical composition of the slab comprises, by mass%,
C: 0.06 to 0.30%,
Si: 0.01 to 2.50%,
Mn: 1.00 to 3.50%,
Ti: 0.001 to 0.100%,
B: 0.0005 to 0.0050%,
P: 0.050% or less,
S: 0.0100% or less,
Al: 1.500% or less,
N: 0.010% or less,
O: 0.0100% or less,
Cr: 0 to 1.00%,
Mo: 0 to 1.00%,
Cu: 0 to 1.00%,
Ni: 0 to 1.00%,
Co: 0 to 1.00%,
W: 0 to 1.00%,
Sn: 0 to 1.00%,
Sb: 0 to 0.50%,
Nb: 0 to 0.200%,
V: 0 to 1.00%,
As: 0 to 0.10%,
Zn: 0 to 1.00%,
Ca: 0 to 0.0100%,
Mg: 0 to 0.0100%,
Ce: 0 to 0.0150%,
Zr: 0 to 0.0100%,
La: 0 to 0.0150%,
Hf: 0 to 0.0100%,
Bi: 0 to 0.0100%,
REM other than Ce and La: 0 to 0.0100%, and
bal.: Fe and impurities.

It should be noted that the preferable contents of the constituents in the chemical composition of the slab etc. are basically the same as the chemical composition of the above-mentioned steel sheet.

In the hot rolling step, the heating temperature of the slab is not particularly limited, but to sufficiently dissolve the borides, carbides, etc., in general it is preferably 1150°C or more. It should be noted that the steel slab used is preferably cast by the continuous casting method from the viewpoint of productivity, but it may also be produced by the ingot making method or thin slab casting method.

### (Rough Rolling)

In the method of production, the heated slab may be rough rolled before the finish rolling so as to adjust the sheet thickness etc. The conditions of such rough rolling are not particularly limited, but from the viewpoint of recrystallization during hot rolling, rough rolling is preferably performed so that the total rolling reduction at 1050°C or more becomes 60% or more. The total rolling reduction may, for example, be 90% or less.

### (Finish Rolling)

Next, the above-mentioned slab is hot rolled by finish rolling to obtain the hot rolled steel sheet. The finish rolling entry side temperature at the finish rolling is not particularly limited, but to make the structure of the hot rolled steel sheet a suitable one, it is preferably 900 to 1050°C. Further, the total rolling reduction at the finish rolling is preferably 70 to 95%.

In the present method of production, to form the above-mentioned deboronized layer, finish rolling is performed by three or more passes, the rolling reduction of the respective passes of the final three passes at the finish rolling is 20% or more, the time between passes is within 1 second, the entry side steel sheet temperature before the final three passes is 1000°C or less, and the finish rolling completion temperature is 850 to 950°C. Further, the time from after the completion of the final pass to the start of cooling is within 3 seconds. If performing the finish rolling under such conditions, the accumulation of strain at the austenite promotes ferrite transformation and causes the surface of the hot rolled steel sheet to soften whereby it is possible to promote the introduction of strain at the surface by the grinding of the next step and, as a result, it is possible to form the above-mentioned deboronized layer at the final product steel sheet. The number of passes of the finish rolling is not particularly limited so long as the final three passes satisfy the above-mentioned conditions.

It should be noted that, in this Description, the "final three passes" means the three passes of the pass of the third pass counted from the final pass, the pass of the second pass and the pass of the first pass from among the three or more passes in the finish rolling.

### (Coiling Temperature: 450 to 650°C)

The hot rolled steel sheet after the above-mentioned finish rolling is coiled after cooling down to a predetermined coiling temperature. At this time, the coiling temperature is 450 to 650°C from the viewpoint of the strength and workability of the hot rolled sheet. The coiling temperature may also be 500°C or more. Further, the coiling temperature may be 620°C or less.

After finishing the coiling, for the purpose of promoting the formation of a deboronized layer at the later explained heat treatment step, it is also possible to add a step of retaining the heat of the coiled hot rolled steel sheet in a heat insulating vessel. As one example of the heat retention step, the hot rolled steel sheet may be placed in a heat insulating vessel with inside walls covered by a heat insulation material so as to retain the heat within 30 minutes after the completion of coiling. At this time, the heat retention conditions may be a peak temperature of the atmosphere inside the vessel of 500 to 650°C and a time until the temperature of the atmosphere reaches the above peak temperature of 1 to 8 hours. If retaining the heat under such conditions, the surface layer part of the hot rolled steel sheet further softens, introduction of strain in the following grinding step is promoted, and formation of a deboronized layer at the later explained heat treatment step is further promoted, whereby the bendability after plastic working the finally obtained steel sheet can be further improved.

### [Grinding Step (e)]

Next, the front and back surfaces of the coiled steel sheet are ground using a rotary grinding brush in the grinding step (e). As the brush able to be used in the grinding step, for example, D-100-33 made by Hotani etc. may be mentioned. The grinding conditions are a rotational speed R (rpm) of the grinding brush, diameter D (m) of the grinding brush, and the running speed V (m/min) of the steel sheet are set to satisfy the following formula (5). If grinding under conditions satisfying such a formula (5), by strain being introduced in the surface layer part of the steel sheet, diffusion of boron is promoted at the later explained heat treatment step and the deboronized layer formed at the later explained heat treatment step is expanded.
[Mathematical 2] $\frac{R ⋅ D}{V} > 1 0$

It should be noted that in formula (5), (R·D)/V may be 11 or more, 13 or more, or 15 or more. Further, the upper limit of the (R·D)/V is not particularly limited, but (R·D)/V may be 60 or less, 55 or less, or 50 or less.

Such a step (e) has to be performed at a time from the completion of the hot rolling to before the cold rolling. It may be performed at a timing of either before the later explained pickling step or after the pickling step.

### [Pickling Step (b)]

Next, the steel sheet after the hot rolling step (a) or the grinding step (e) is pickled in the pickling step (b). The method of pickling in the pickling step may be based on an ordinary method. Further, in the pickling step, skin pass rolling may be performed for correction of the shape of the hot rolled coil and improvement of pickling ability.

### [Cold Rolling Step (c)]

Next, the steel sheet after the pickling step (b) or the grinding step (e) is cold rolled in the cold rolling step (c). In the cold rolling step, the rolling reduction of the cold rolling is 30 to 75% considering the accumulation of strain and the burden on the cold rolling mill due to the rolling load. For example, the rolling reduction may be 40% or more. Further, the rolling reduction may be 70% or less or 60% or less.

### [Heat Treatment Step (d)]

Next, the steel sheet obtained at the cold rolling step (c) is heat treated in a heat treatment step (d). The heat treatment step is comprised of a successively performed step (d-1) of heating the steel sheet obtained at step (c) from 650°C to the Ac1+50°C or more and 950°C or less maximum heating temperature by an average heating speed of 0.5 to 500°C/s, a step (d-2) of holding the steel sheet at the maximum heating temperature for 1 to 300 seconds, a step (d-3) of cooling the steel sheet down to an Ms point (martensite transformation point)-100°C or less temperature in which the cooling from 700°C to 500°C is performed by cooling by a 10°C/s or more average cooling speed, and a step (d-4) of holding the steel sheet at 200 to 350°C for 1 to 600 seconds.

The deboronation can be made to sufficiently proceed by controlling the hot rolling conditions as explained above to soften the surface layer part of the steel sheet, introducing a large amount of strain at the surface layer part of the steel sheet at the grinding step, and further making the H₂O in the atmosphere and the B of the surface of the steel sheet react to form oxides in the above step (d-1) to step (d-4) of the heat treatment step, i.e., the temperature raising and soaking step.

At the above-mentioned step (d-1), the average heating speed up to the maximum heating temperature is 0.5 to 500°C/s from the viewpoint of causing recrystallization of ferrite to proceed and suppressing coarsening of austenite. The average heating speed may also be 1.0°C/s or more or 2.0°C/s or more. Further, the average heating speed may also be 400°C/s or less or 300°C/s or less. In this case, the "average heating speed" means the value obtained by dividing the difference between 650°C and the maximum heating temperature by the time required for reaching the maximum heating temperature from 650°C.

At the above-mentioned step (d-1), the maximum heating temperature is Ac1+50°C or more and 950°C or less from the viewpoint of progression of austenization and suppression of coarsening of the austenite size. Further, at the above-mentioned step (d-2), the holding time at the maximum heating temperature is 1 to 300 seconds from the viewpoint of progression of the austenization and the productivity. While holding at the maximum heating temperature, the steel sheet does not necessarily have to be held at a constant temperature. The temperature may fluctuate within the range of the above maximum heating temperature. In this case, "holding" means maintaining the temperature within a range not exceeding the predetermined upper and lower limits at a predetermined temperature±20°C, preferably within a range of ±10°C.

After holding at the maximum heating temperature, at the above-mentioned step (d-3), the steel sheet is cooled down to the Ms point-100°C or less temperature, but at this time, from 700°C to 500°C, the steel sheet is cooled by a 10°C/s or more average cooling speed. The average cooling speed from 700°C to 500°C may be 20°C/s or more, 30°C/s or more, or 50°C/s or more.

To obtain the desired structure, after cooling down to the Ms point-100°C or less temperature, at the above-mentioned step (d-4), the steel sheet is held at 200 to 350°C for 1 to 600 seconds. The "holding" at this step (d-4), in the same way as above, does not require holding at a certain temperature. It means holding at the predetermined temperature±20°C, preferably within ±10°C in range.

At the above-mentioned step (d-4), the holding operation at the 200 to 350°C temperature region may be performed by performing the cooling down to the Ms point-100°C or less down to less than 200°C, then reheating. Alternatively, if the end temperature of the cooling down to the Ms point-100°C or less is 200°C or more, it may also be performed in the middle of the cooling process next performed.

Further, at the above-mentioned step (d-1), the atmosphere in the surroundings of the steel sheet when heating from 650°C to the maximum heating temperature is controlled so that the steam partial pressure pH₂O and the hydrogen partial pressure pH₂ satisfy the following formula (6). If the log(pH₂O/pH₂) in formula (6) is less than -1.0, the decarburization reaction does not sufficiently proceed and the desired maximum bending angle after imparting 2% prestrain and the effect of suppression of the load drop are not obtained. Further, if the log(pH₂O/pH₂) in formula (6) is more than -0.1, the effect of improvement of bending becomes saturated and the strength of the steel sheet is liable to fall.
$- 1.0 \leq log \left({pH}_{2}O/{pH}_{2}\right) \leq - 0.1$
pH₂O: steam partial pressure
pH₂: hydrogen partial pressure

It should be noted that the log(pH₂O/pH₂) in formula (6) may be -0.9 or more or -0.8 or more. Further, the log(pH₂O/pH₂) in formula (6) may be -0.2 or less or -0.3 or less.

As explained above, the steel sheet of the present invention may be formed with a plating layer at its surface. The plating layer can, for example, be a hot dip galvanized layer. Further, in accordance with need, after formation of the hot dip galvanized layer, the layer may be alloyed to form a hot dip galvannealed layer. The plating layer may be formed and the alloying may be performed in accordance with ordinary methods and are not particularly limited. The plating can be performed in the middle of cooling from the maximum heating temperature to a temperature of the Ms point-100°C or less. In this case, the cooling may be ended once at the plating temperature and then after the plating ends, the cooling performed down to a temperature of the Ms point-100°C or less by a 10°C/s or more average cooling speed.

By the above method of production, it is possible to obtain the steel sheet of the present invention excellent in tensile strength and excellent in bendability after plastic working. The bendability is evaluated by imparting 2% prestrain to a test piece taken from the steel sheet to be evaluated, then performing a bending test by the method prescribed in the Verband der Automobilindustrie (VDA) standard 238-100 and comparing the maximum bending angle (α) obtained from the test. The load drop after the maximum load is evaluated by reading the α+5 degree load, dividing the α+5 degree load by the maximum load, and comparing the values (=α+5 degree load/maximum bending load). Note that, at the time of evaluation, the reason for imparting a 2% prestrain is because the steel sheet of the present invention is envisioned as being used as a part.

### EXAMPLES

Next, an embodiment of the present invention will be explained. The conditions in this embodiment are one example of the conditions employed for confirming the feasibility and effects of the present invention. The present invention is not limited to this example of the conditions. The present invention can employ various conditions so long as not departing from the gist of the present invention and achieving the object of the present invention.

Steels having various chemical compositions were cast to prepare slabs. These slabs were used for hot rolling to produce hot rolled steel sheets. Further, the hot rolled steel sheets were successively ground down, cold rolled, and heat treated to produce cold rolled steel sheets.

Some of the obtained cold rolled steel sheets were plated. Samples taken from the obtained steel sheets were analyzed for chemical composition, whereupon it was confirmed that there were no changes from the chemical compositions of the slabs. The chemical compositions of these steel sheets are shown in Table 1. The balances besides the constituents shown in Table 1 are Fe and impurities. It should be noted that, for plated steel sheets, the chemical compositions are those of the base steel sheets with the plating layers at the surfaces peeled off under the above conditions. The underlines attached to the chemical compositions in Table 1 show values outside the scope of the present invention.

### [Table 2]

**Table 2**

| No. | Steel type | Hot rolling step: Step (a) | | | | | | | | | | | |
|---|---|---|---|---|---|---|---|---|---|---|---|---|---|
| | | Slab heating temp. | Finish rolling | | | | | | | | Coiling temp. | Heat ins./ retention | 500 to 650°C time |
| | | | R1 entry side temp. | R1 | t1 | R2 | t2 | R3 | t3 | R3 exit side temp. | | | |
| | | °C | °C | % | sec | % | sec | % | sec | °C | °C | °C | h |
| 1 | A | 1236 | 923 | 28 | 0.8 | 26 | 0.6 | 21 | 1.6 | 885 | 584 | - | - |
| 2 | A | 1232 | 926 | 24 | 0.7 | 25 | 0.5 | 24 | 1.9 | 906 | 542 | Yes | 2.3 |
| 3 | A | 1212 | 934 | 23 | 0.5 | 27 | 0.7 | 22 | 2.1 | 879 | 603 | - | - |
| 4 | A | 1245 | 964 | 22 | 0.6 | 24 | 0.7 | 26 | 1.9 | 901 | 594 | - | - |
| 5 | A | 1256 | 958 | 12 | 0.7 | 22 | 0.4 | 24 | 2.2 | 942 | 573 | - | - |
| 6 | A | 1237 | 936 | 29 | 0.3 | 28 | 0.9 | 14 | 2.7 | 910 | 522 | - | - |
| 7 | A | 1220 | 997 | 26 | 0.7 | 22 | 0.6 | 32 | 2.4 | 908 | 546 | - | - |
| 8 | A | 1221 | 954 | 27 | 0.5 | 21 | 0.9 | 25 | 2.1 | 932 | 573 | - | - |
| 9 | A | 1222 | 941 | 23 | 0.4 | 29 | 0.8 | 27 | 2.5 | 905 | 517 | - | - |
| 10 | A | 1210 | 954 | 22 | 0.3 | 28 | 0.8 | 30 | 2.6 | 936 | 637 | - | - |
| 11 | B | 1268 | 940 | 26 | 0.5 | 25 | 0.8 | 24 | 1.1 | 909 | 533 | - | - |
| 12 | B | 1215 | 981 | 28 | 0.4 | 23 | 0.7 | 29 | 1.6 | 915 | 523 | Yes | 3.2 |
| 13 | B | 1231 | 924 | 25 | 0.4 | 29 | 0.4 | 24 | 2.1 | 912 | 555 | - | - |
| 14 | B | 1215 | 915 | 22 | 0.6 | 26 | 0.5 | 27 | 2.6 | 891 | 546 | - | - |
| 15 | B | 1259 | 954 | 23 | 0.3 | 21 | 0.6 | 27 | 2.4 | 921 | 641 | - | - |
| 16 | B | 1215 | 981 | 28 | 0.4 | 23 | 0.7 | 29 | 1.6 | 915 | 523 | - | - |
| 17 | C | 1223 | 959 | 27 | 0.4 | 21 | 0.5 | 22 | 1.7 | 897 | 615 | - | - |
| 18 | D | 1254 | 964 | 22 | 0.5 | 26 | 0.4 | 22 | 2.3 | 920 | 595 | - | - |
| 19 | E | 1236 | 954 | 22 | 0.7 | 21 | 0.4 | 29 | 1.6 | 912 | 605 | - | - |
| 20 | F | 1278 | 931 | 22 | 0.8 | 27 | 0.5 | 21 | 1.7 | 894 | 625 | - | - |
| 21 | G | 1247 | 960 | 21 | 0.4 | 29 | 0.5 | 25 | 2.6 | 887 | 561 | - | - |
| 22 | H | 1232 | 968 | 28 | 0.8 | 24 | 0.4 | 29 | 2.2 | 918 | 590 | - | - |
| 23 | I | 1234 | 948 | 24 | 0.3 | 22 | 0.7 | 20 | 2.6 | 896 | 547 | - | - |
| 24 | J | 1253 | 951 | 22 | 0.6 | 29 | 0.5 | 24 | 2.1 | 925 | 594 | - | - |
| 25 | K | 1242 | 957 | 21 | 0.4 | 26 | 0.6 | 25 | 2.3 | 893 | 620 | - | - |
| 26 | L | 1278 | 967 | 26 | 0.3 | 25 | 0.9 | 24 | 2.2 | 926 | 611 | - | - |
| 27 | M | 1262 | 911 | 24 | 0.7 | 27 | 0.6 | 26 | 2.7 | 891 | 554 | - | - |
| 28 | N | 1218 | 957 | 27 | 0.9 | 21 | 0.6 | 32 | 2.1 | 923 | 556 | - | - |
| 29 | O | 1221 | 936 | 23 | 0.5 | 26 | 0.3 | 25 | 1.5 | 899 | 583 | - | - |
| 30 | P | 1275 | 928 | 22 | 0.7 | 27 | 0.6 | 29 | 2.7 | 910 | 603 | - | - |

The hot rolling was performed under the conditions described in Table 2. In Table 2, the "R1 entry side temperature" means the entry side steel sheet temperature of the third pass counted from the final pass of the finish rolling. "R1" means the rolling reduction of the third pass counted from the final pass. R2 means the rolling reduction of the second pass counted from the final pass. R3 means the rolling reduction of the final pass. Further, t1 means the time from the end of the third pass counted from the final pass to the start of the second pass counted from the final pass. t2 means the time from the end of the second pass counted from the final pass to the start of the final pass. t3 means the time from the end of the final pass to the start of the cooling. Further, the R3 exit side temperature means the temperature of the steel sheet at the time of the end of the final pass, i.e., the finish rolling completion temperature.

After that, a rotary grinding brush containing abrasives was used to grind the front and back surfaces of the hot rolled steel sheet. The grinding conditions are found from a rotational speed R (rpm) of the grinding brush, diameter D (m) of the grinding brush, and running speed V (m/min) of the steel sheet, They were set so that the value of (R·D)/V became the values shown in Table 3. Next, the ground steel sheet was pickled. Further, the pickled steel sheet was cold rolled by the rolling reduction described in Table 3.

After that, the cold rolled steel sheet was heat treated. The heat treatment comprised heating up to the maximum heating temperature, then holding it there and cooling. The sheet was cooled down to the Ms point-100°C or less in temperature, then holding at 200 to 350°C. The No. 15 steel sheet with a cooling end temperature down to the Ms point-100°C or less higher than the 200 to 350°C holding temperature was held by a cooling process after finishing cooling down to the Ms point-100°C or less. The steel sheets other than No. 15 were reheated to a predetermined temperature after finishing cooling it down to the Ms point-100°C or less temperature and then held there. The values of these conditions and the value of the log(pH₂O/pH₂) from 650°C to the maximum heating temperature are shown in Table 3. In this case, pH₂O is the steam partial pressure, while pH₂ is the hydrogen partial pressure. Further, in Table 3, Ms is the martensite transformation point (°C) of the steel used.

It should be noted that, in Table 3, the Ac1 point (°C), which is the standard for the setting range of the maximum heating temperature of the heat treatment, was found in accordance with the following formula. The Ac1 points of the steel sheets are shown in Table 1. $Ac 1 = 723 - 10.7 \left[Mn\right] - 16.9 \left[Ni\right] + 29.1 \left[Si\right] + 16.9 \left[Cr\right]$

In the above formula, [Mn], [Ni], [Si], and [Cr] mean the contents (mass%) of the elements.

Further, in Table 3, the Ms point (°C) is found in accordance with the following formula: $Ms = 561 - 474 \left[C\right] - 33 \left[Mn\right] - 7.5 \left[Si\right] - 17 \left[Cr\right] - 17 \left[Ni\right] - 21 \left[Mo\right] + 10 \left[Co\right]$

In the above formula, [C], [Mn], [Si], [Cr], [Ni], [Mo], and [Co] mean the contents (mass%) of the elements.

After that, some of the steel sheets were continuously hot dip galvanized and further some were alloyed. The plating conditions were not special ones and could be known general conditions. In Table 3, "GA" means hot dip galvannealed steel sheet. Further, "GI" means hot dip galvanized steel sheet hot dip galvanized steel sheet which has not been alloyed. "CR" means cold rolled steel sheet which has not been plated.

It should be noted that the underlines attached to the various numerical values in Table 2 and Table 3 show outside the scope of the present invention, production conditions not yielding the steel sheet of the present invention, or various properties of steel sheet which are not preferable.

### [Table 3]

**Table 3**

| No. | Grinding step: step (e) | Cold rolling step: step (c) | Heat treatment step: step (d) | | | | | | | | Ms point | Grade |
|---|---|---|---|---|---|---|---|---|---|---|---|---|
| | (R·D)/V | Rolling reduction | Heating speed | Max. heating temp. | log(pH₂O/ pH₂) | Holding time at max. heating temp. | Average cooling speed from 700°C to 500°C | End temp. of cooling from Ms point-100°C or less | Holding temp. at 200 to 350°C | Holding time. at 200 to 350°C | | |
| | | % | °C/s | °C | - | sec | °C/s | °C | °C | sec | °C | |
| 1 | 16 | 60 | 2.2 | 819 | -0.5 | 92 | 56 | 208 | 276 | 359.0 | 419 | CR |
| 2 | 21 | 60 | 2.0 | 825 | -0.5 | 99 | 61 | 198 | 261 | 378.0 | 419 | CR |
| 3 | 18 | 60 | 2.1 | 871 | -0.7 | 94 | 55 | 251 | 304 | 405.0 | 419 | GA |
| 4 | 22 | 60 | 1.9 | 836 | -0.3 | 91 | 57 | 215 | 295 | 369.0 | 419 | GI |
| 5 | 17 | 60 | 1.9 | 857 | -0.7 | 84 | 71 | 291 | 345 | 259.0 | 419 | CR |
| 6 | 23 | 60 | 2.1 | 844 | -0.4 | 130 | 54 | 264 | 303 | 211.0 | 419 | CR |
| 7 | None | 60 | 2.3 | 871 | -0.7 | 91 | 51 | 312 | 311 | 278.0 | 419 | CR |
| 8 | 21 | 60 | 2.1 | 753 | -0.5 | 123 | 53 | 243 | 327 | 217.0 | 419 | CR |
| 9 | 24 | 60 | 1.9 | 814 | -2.0 | 102 | 67 | 257 | 340 | 219.0 | 419 | CR |
| 10 | 24 | 60 | 1.9 | 812 | -0.7 | 114 | 61 | 140 | 167 | 242.0 | 419 | CR |
| 11 | 22 | 60 | 2.2 | 853 | -0.3 | 117 | 54 | 209 | 239 | 412.0 | 350 | CR |
| 12 | 31 | 60 | 2.4 | 851 | -0.6 | 112 | 76 | 231 | 307 | 245.0 | 350 | CR |
| 13 | 18 | 60 | 2.0 | 840 | -0.5 | 109 | 57 | 201 | 247 | 365.0 | 350 | GA |
| 14 | 29 | 60 | 2.1 | 846 | -0.7 | 85 | 51 | 215 | 245 | 367.0 | 350 | GI |
| 15 | 26 | 60 | 2.1 | 867 | -0.4 | 118 | 64 | 326 | 341 | 274.0 | 350 | CR |
| 16 | 4 | 60 | 2.4 | 881 | -0.5 | 112 | 71 | 228 | 307 | 245.0 | 350 | CR |
| 17 | 37 | 60 | 2.1 | 876 | -0.6 | 81 | 62 | 291 | 302 | 221.0 | 445 | CR |
| 18 | 29 | 60 | 2.0 | 840 | -0.5 | 105 | 51 | 216 | 311 | 276.0 | 361 | CR |
| 19 | 26 | 60 | 2.1 | 836 | -0.6 | 90 | 56 | 269 | 276 | 351.0 | 421 | CR |
| 20 | 23 | 60 | 2.0 | 842 | -0.3 | 128 | 55 | 213 | 297 | 235.0 | 338 | CR |
| 21 | 28 | 60 | 1.8 | 843 | -0.5 | 87 | 64 | 286 | 301 | 231.0 | 422 | CR |
| 22 | 31 | 60 | 2.2 | 821 | -0.6 | 126 | 71 | 222 | 307 | 270.0 | 330 | CR |
| 23 | 24 | 60 | 2.0 | 864 | -0.6 | 124 | 54 | 286 | 326 | 224.0 | 426 | CR |
| 24 | 30 | 60 | 2.3 | 842 | -0.4 | 102 | 72 | 203 | 278 | 260.0 | 350 | CR |
| 25 | 22 | 60 | 1.9 | 864 | -0.4 | 119 | 55 | 222 | 304 | 229.0 | 465 | CR |
| 26 | 32 | 60 | 2.4 | 818 | -0.5 | 106 | 52 | 128 | 312 | 246.0 | 285 | CR |
| 27 | 12 | 60 | 2.3 | 887 | -0.7 | 130 | 54 | 245 | 345 | 228.0 | 375 | CR |
| 28 | 31 | 60 | 2.1 | 876 | -0.5 | 97 | 63 | 336 | 346 | 243.0 | 477 | CR |
| 29 | 41 | 60 | 2.3 | 833 | -0.7 | 90 | 63 | 219 | 271 | 239.0 | 329 | CR |
| 30 | 42 | 60 | 2.0 | 861 | -0.8 | 118 | 61 | 254 | 310 | 227.0 | 390 | CR |

The obtained steel sheets were measured for emission intensities of B of B30, B140, and B150 at the different depth positions of 30 µm, 140 µm, and 150 µm from the steel sheet surface when using the method of the above-mentioned high frequency glow discharge spectrometry (high frequency GDS analysis) for measurement by the above-mentioned high frequency GDS analysis in the sheet thickness direction from the steel sheet surface. Simultaneously the emission intensities of C of C30, C140, and C150 at the different depth positions of 30 µm, 140 µm, and 150 µm from the steel sheet surface were measured. These measurement results are shown in the following Table 4.

Further, from the center part of width of the obtained steel sheet, a No. 5 tensile test piece of JIS Z 2241: 2011 having a direction perpendicular to the rolling direction as its longitudinal direction was taken and that test piece was used to perform a tensile test based on JIS Z2241: 2011 to measure the tensile strength (TS). It should be noted that, regarding the No. 3, 4, 13 and 14 steel sheets, the tensile strength as plated was measured without peeling off the plating from the plated steel sheets. In the present embodiment, the basis of the tensile strength (1180 MPa or more) was made the same as the steel sheet which was not plated. The measurement results of the tensile strength of the steel sheet are shown in the following Table 4.

Further, from the center part of width of the obtained steel sheet, a tensile test piece of a parallel part width of 30 mm having a direction perpendicular to the rolling direction as its longitudinal direction was taken. 2% prestrain was imparted, then a rectangular sample of a width 30 mm x length 60 mm was taken from the parallel part. Next, to simulate a painting and baking step of an automobile, heat treatment was performed at 170°C for 20 minutes. The heat treated test piece was subjected to a bending test by the method prescribed in the Verband der Automobilindustrie (VDA) standard 238-100. The maximum bending angle (α) was measured. Regarding the measurement results, a maximum bending angle of 60 degrees or more was judged excellent in bendability. The bending direction was determined so that the rolling direction became parallel to the bending ridgeline. It should be noted that in the No. 3, 4, 13, and 14 steel sheets, the maximum bending angle as plated was measured without peeling off the plating from the plated steel sheet. In this embodiment, the basis of the maximum bending angle (60 degrees or more) was made the same as steel sheet not formed with a plating.

Furthermore, the load drop was evaluated by reading the α+5 degree load, dividing the α+5 degree load by the maximum load (=α+5 degree load/maximum bending load), and using the value for evaluation. In other words, the larger the numerical value, the smaller the load. If the numerical value was 0.50 or more, the bendability was judged as good.

It should be noted that in evaluating the "bendability" of the steel sheets, samples where the above-mentioned maximum bending angle was 60 degrees or more and the value of the load of the above-mentioned load drop of α+5 degrees divided by the maximum load was 0.50 or more were judged as being "excellent in bendability".

The results of measurement of the maximum bending angle and load drop of the steel sheet are shown in the following Table 4.

In this case, the points to note in the evaluation of the present invention will be explained. The features of the present invention, i.e., the chemical composition, steel structure, B concentration distribution, C concentration distribution, and other features of the steel sheet, are prescribed for regions unrelated to any surface covering. On the other hand, the mechanical properties of steel sheet (i.e., the tensile strength and bendability) are generally believed to change somewhat depending on any surface covering. Even under such a situation, in the present invention, steel sheet of the same surface conditions as the point of time of use of the steel sheet is used to judge whether the mechanical properties of the steel sheet fall in the scope of the present invention. This is because for a person using steel sheet with a covered surface, not the mechanical properties of the state with the covering peeled off, but the mechanical properties in the covered state are important. Accordingly, in the invention examples, plated steel sheets (No. 3, 4, 13, and 14 steel sheets) are evaluated for the mechanical properties of tensile strength and bendability (maximum bending angle and load drop) in the state as plated while not plated steel sheets (steel sheets other than No. 3, 4, 13, and 14) are evaluated in the non-plated state.

It should be noted that in Table 4, "α" in the microstructure means ferrite. Further, "TM" means tempered martensite. "FM" means fresh martensite. "y" means retained austenite. "P+θ" means the total of pearlite and cementite. Further, "B" means bainite.

In Table 4, the underlines given to various numerical values etc. indicate outside the scope of the present invention, production conditions not yielding the steel sheet of the present invention, or properties of the steel sheet which are not preferable.

### [Table 4]

**Table 4**

| No. | Steel type | Microstructure | | | | | | Surface | | | | Mechanical properties | | | Remarks |
|---|---|---|---|---|---|---|---|---|---|---|---|---|---|---|---|
| | | α | TM | γ | FM | P +θ | B | B30 /B150 | C30 /C150 | B140 /B150 | C140 /C150 | Tensile strength | Max. bending angle | Load reduction | |
| | | % | % | % | % | % | % | - | - | - | - | MPa | ○ | - | |
| 1 | A | 18 | 54 | 5 | 2 | 0 | 21 | 0.65 | 0.28 | 0.97 | 1.01 | 1229 | 83 | 0.56 | Inv. ex. |
| 2 | A | 14 | 61 | 4 | 3 | 0 | 18 | 0.21 | 0.34 | 0.98 | 0.97 | 1268 | 96 | 0.86 | Inv. ex. |
| 3 | A | 9 | 49 | 6 | 5 | 0 | 31 | 0.69 | 0.39 | 1.02 | 0.99 | 1209 | 85 | 0.61 | Inv. ex. |
| 4 | A | 16 | 56 | 4 | 4 | 0 | 20 | 0.74 | 0.31 | 0.99 | 0.99 | 1231 | 82 | 0.64 | Inv. ex. |
| 5 | A | 11 | 54 | 6 | 8 | 0 | 21 | 0.94 | 0.43 | 0.96 | 0.93 | 1236 | 53 | 0.11 | Comp. ex. |
| 6 | A | 11 | 74 | 2 | 3 | 0 | 10 | 0.92 | 0.46 | 1.04 | 1.02 | 1247 | 55 | 0.16 | Comp. ex. |
| 7 | A | 2 | 43 | 8 | 7 | 0 | 40 | 0.97 | 0.34 | 0.99 | 0.98 | 1183 | 43 | 0.23 | Comp. ex. |
| 8 | A | 42 | 24 | 6 | 7 | 0 | 21 | 0.72 | 0.44 | 1.00 | 0.96 | 1032 | 97 | 0.78 | Comp. ex. |
| 9 | A | 13 | 57 | 5 | 4 | 0 | 21 | 0.64 | 0.93 | 1.00 | 0.99 | 1231 | 83 | 0.13 | Comp. ex. |
| 10 | A | 23 | 54 | 2 | 16 | 0 | 5 | 0.59 | 0.36 | 0.97 | 0.99 | 1296 | 52 | 0.31 | Comp. ex. |
| 11 | B | 0 | 95 | 2 | 3 | 0 | 0 | 0.65 | 0.31 | 0.99 | 1.01 | 1521 | 74 | 0.64 | Inv. ex. |
| 12 | B | 0 | 92 | 3 | 5 | 0 | 0 | 0.18 | 0.34 | 1.00 | 1.02 | 1493 | 91 | 0.88 | Inv. ex. |
| 13 | B | 0 | 96 | 2 | 2 | 0 | 0 | 0.66 | 0.41 | 1.03 | 0.97 | 1512 | 76 | 0.65 | Inv. ex. |
| 14 | B | 0 | 93 | 3 | 4 | 0 | 0 | 0.46 | 0.36 | 0.99 | 1.01 | 1516 | 77 | 0.67 | Inv. ex. |
| 15 | B | 0 | 23 | 3 | 19 | 0 | 55 | 0.60 | 0.42 | 0.97 | 1.00 | 1243 | 54 | 0.07 | Comp. ex. |
| 16 | B | 0 | 91 | 4 | 5 | 0 | 0 | 0.91 | 0.34 | 1.00 | 1.02 | 1512 | 57 | 0.12 | Comp. ex. |
| 17 | C | 26 | 69 | 2 | 1 | 0 | 2 | 0.58 | 0.35 | 1.00 | 0.93 | 1191 | 89 | 0.68 | Inv. ex. |
| 18 | D | 2 | 87 | 4 | 3 | 2 | 2 | 0.56 | 0.19 | 0.97 | 0.99 | 1523 | 67 | 0.54 | Inv. ex. |
| 19 | E | 12 | 68 | 3 | 5 | 0 | 12 | 0.67 | 0.24 | 0.99 | 1.03 | 1216 | 81 | 0.55 | Inv. ex. |
| 20 | F | 0 | 91 | 7 | 1 | 0 | 1 | 0.45 | 0.36 | 1.00 | 0.99 | 1536 | 63 | 0.55 | Inv. ex. |
| 21 | G | 28 | 61 | 2 | 3 | 0 | 6 | 0.70 | 0.41 | 0.99 | 1.00 | 1186 | 86 | 0.68 | Inv. ex. |
| 22 | H | 0 | 93 | 1 | 2 | 0 | 4 | 0.72 | 0.33 | 0.96 | 0.98 | 1534 | 65 | 0.54 | Inv. ex. |
| 23 | I | 8 | 52 | 4 | 2 | 0 | 34 | 0.67 | 0.36 | 1.00 | 0.99 | 1268 | 80 | 0.58 | Inv. ex. |
| 24 | J | 8 | 78 | 5 | 5 | 0 | 4 | 0.61 | 0.24 | 1.02 | 0.99 | 1472 | 71 | 0.78 | Inv. ex. |
| 25 | K | 36 | 45 | 8 | 2 | 0 | 9 | 0.55 | 0.44 | 1.00 | 0.96 | 1059 | 91 | 0.84 | Comp. ex. |
| 26 | L | 2 | 75 | 12 | 6 | 4 | 1 | 0.59 | 0.47 | 0.97 | 1.02 | 1489 | 63 | 0.08 | Comp. ex. |
| 27 | M | 10 | 45 | 9 | 3 | 0 | 33 | 0.65 | 0.33 | 1.00 | 0.99 | 1346 | 64 | 0.12 | Comp. ex. |
| 28 | N | 33 | 52 | 3 | 2 | 0 | 10 | 0.68 | 0.46 | 1.01 | 0.98 | 1021 | 88 | 0.79 | Comp. ex. |
| 29 | O | 0 | 84 | 11 | 3 | 0 | 2 | 0.63 | 0.37 | 0.98 | 1.00 | 1503 | 56 | 0.14 | Comp. ex. |
| 30 | P | 34 | 48 | 4 | 9 | 0 | 5 | - | 0.45 | 1.01 | 0.98 | 1089 | 78 | 0.59 | Comp. ex. |

In the No. 5 steel sheet, the rolling reduction of the third pass from the final pass of the finishing rolling at the hot rolling step was low and a suitable deboronized layer was not formed, and therefore the result was the bendability was poor.

In the No. 6 steel sheet, the rolling reduction of the final pass of the finishing rolling at the hot rolling step was low and a suitable deboronized layer was not formed, and therefore the result was the bendability was poor.

In the No. 7 steel sheet, a brush was not used for grinding and a suitable deboronized layer was not formed, and therefore the result was the bendability was poor.

In the No. 8 steel sheet, the maximum heating temperature of the heat treatment step was low, therefore the ferrite fraction was high and the fraction of the tempered martensite became low, and therefore the desired tensile strength could not be obtained.

In the No. 9 steel sheet, the log(pH₂O/pH₂) of the heat treatment step was smaller than -1.0 and a suitable decarburized layer was not formed, and therefore while the maximum bending angle was large, the load in the case of exceeding the maximum bending angle became small.

In the No. 10 steel sheet, the holding temperature after cooling at the heat treatment step was low and the fraction of fresh martensite became high, and therefore the result was the bendability was poor.

In the No. 15 steel sheet, the cooling end temperature in the heat treatment step was high, the fraction with the fresh martensite was high, and the fraction of the tempered martensite became low, and therefore the result was the bendability was poor.

In the No. 16 steel sheet, the conditions of the grinding step were not suitable and a suitable deboronized layer was not formed, therefore the result was the bendability was poor.

In the No. 25 steel sheet, the C content of the chemical composition was low and the ferrite fraction became high, and therefore the desired tensile strength could not be obtained.

In the No. 26 steel sheet, the C content of the chemical composition was high and the fraction of the retained austenite became high, and therefore while the maximum bending angle was large, the load in the case of exceeding the maximum bending angle became smaller.

In the No. 27 steel sheet, the Si content of the chemical composition was high and the retained austenite fraction became high, and therefore the maximum bending angle was large, but the load when the maximum bending angle was exceeded became small.

In the No. 28 steel sheet, the Mn content of the chemical composition was low and the ferrite fraction became high, and therefore the desired tensile strength could not be obtained.

In the No. 29 steel sheet, the Mn content of the chemical composition was high and the retained austenite fraction became high, and therefore the result was the bendability was poor.

In the No. 30 steel sheet, the B content of the chemical composition was low and the ferrite fraction became high, and therefore the desired tensile strength could not be obtained. It should be noted that the B content was low and the "deboronized layer" could not be identified, and therefore the entry in the field of B30/B150 was made "-".

### REFERENCE SIGNS LIST

1. plated steel sheet
2. base steel sheet
3. plating layer
S_{d}. steel sheet surface
P_{S}. surface layer part
P_{B}. deboronized layer
P₃₀. depth position of 30 µm from steel sheet surface
P₁₅₀. depth position of 150 µm from steel sheet surface

## Claims

1. Steel sheet, in which steel sheet,
a chemical composition of the steel sheet contains, by mass%,
C: 0.06 to 0.30%,
Si: 0.01 to 2.50%,
Mn: 1.00 to 3.50%,
Ti: 0.001 to 0.100%,
B: 0.0005 to 0.0050%,
P: 0.050% or less,
S: 0.0100% or less,
Al: 1.500% or less,
N: 0.010% or less,
O: 0.0100% or less,
Cr: 0 to 1.00%,
Mo: 0 to 1.00%,
Cu: 0 to 1.00%,
Ni: 0 to 1.00%,
Co: 0 to 1.00%,
W: 0 to 1.00%,
Sn: 0 to 1.00%,
Sb: 0 to 0.50%,
Nb: 0 to 0.200%,
V: 0 to 1.00%,
As: 0 to 0.10%,
Zn: 0 to 1.00%,
Ca: 0 to 0.0100%,
Mg: 0 to 0.0100%,
Ce: 0 to 0.0150%,
Zr: 0 to 0.0100%,
La: 0 to 0.0150%,
Hf: 0 to 0.0100%,
Bi: 0 to 0.0100%,
a REM other than Ce and La: 0 to 0.0100%, and
bal.: Fe and impurities,
a steel structure in a range of a 1/8 depth position to 3/8 depth position of a sheet thickness of the steel sheet comprises, by area%,
ferrite: 30% or less,
tempered martensite: 40% or more,
retained austenite: 8% or less,
fresh martensite: 10% or less,
total of pearlite and cementite: 5% or less, and
bal.: bainite,
a surface layer part of the steel sheet has a deboronized layer with an emission intensity of B, measured by high frequency glow discharge spectrometry in a depth direction from a steel sheet surface, satisfying following formula (1) and formula (2),
further, the surface layer part of the steel sheet has an emission intensity of C, measured by high frequency glow discharge spectrometry in the depth direction from the steel sheet surface, satisfying following formula (3) and formula (4), and
a tensile strength is 1180 MPa or more: $B 30 / B 150 < 0.90$ $0.90 \leq B 140 / B 150 \leq 1.10$ where,
B30: emission intensity of B at depth position of 30 µm from the steel sheet surface
B 140: emission intensity of B at depth position of 140 µm from the steel sheet surface
B150: emission intensity of B at depth position of 150 µm from the steel sheet surface $C 30 / C 150 \leq 0.50$ $0.90 \leq C 140 / C 150 \leq 1.10$ where,
C30: emission intensity of C at depth position of 30 µm from the steel sheet surface
C140: emission intensity of C at depth position of 140 µm from the steel sheet surface
C150: emission intensity of C at depth position of 150 µm from the steel sheet surface

2. The steel sheet according to claim 1, wherein the steel sheet surface has a hot dip galvanized layer or a hot dip galvannealed layer.

3. A method of production of steel sheet, which method of production of steel sheet comprising
a hot rolling step (a) of hot rolling a slab having a chemical composition comprising, by mass%,
C: 0.06 to 0.30%,
Si: 0.01 to 2.50%,
Mn: 1.00 to 3.50%,
Ti: 0.001 to 0.100%,
B: 0.0005 to 0.0050%,
P: 0.050% or less,
S: 0.0100% or less,
Al: 1.500% or less,
N: 0.010% or less,
O: 0.0100% or less,
Cr: 0 to 1.00%,
Mo: 0 to 1.00%,
Cu: 0 to 1.00%,
Ni: 0 to 1.00%,
Co: 0 to 1.00%,
W: 0 to 1.00%,
Sn: 0 to 1.00%,
Sb: 0 to 0.50%,
Nb: 0 to 0.200%,
V: 0 to 1.00%,
As: 0 to 0.10%,
Zn: 0 to 1.00%,
Ca: 0 to 0.0100%,
Mg: 0 to 0.0100%,
Ce: 0 to 0.0150%,
Zr: 0 to 0.0100%,
La: 0 to 0.0150%,
Hf: 0 to 0.0100%,
Bi: 0 to 0.0100%,
REM other than Ce and La: 0 to 0.0100%, and
bal.: Fe and impurities at a 850 to 950°C finish rolling end temperature to obtain hot rolled steel sheet, then cooling the hot rolled steel sheet down to 450 to 650°C and coiling the hot rolled steel sheet,
a pickling step (b) of pickling the steel sheet obtained at the hot rolling step (a),
a cold rolling step (c) of cold rolling the steel sheet obtained by the pickling step (b) by a 30 to 75% rolling reduction to obtain a cold rolled steel sheet,
a heat treatment step (d) of heat treating the steel sheet obtained at the cold rolling step (c), and
a grinding step (e), before or after the pickling step (b), of using a rotary type grinding brush containing an abrasive to grind front and back surfaces of the steel sheet obtained at the hot rolling step (a) or the steel sheet obtained at the pickling step (b),
in the hot rolling step (a), finish rolling comprises three passes or more, a rolling reduction of respective passes of final three passes of the finish rolling is 20% or more, a time between passes is within 1 second, an entry side steel sheet temperature before the final three passes is 1000°C or less, and a time from completion of a final pass to start of cooling is within 3 seconds,
in the grinding step (e), a rotational speed R (rpm) of the grinding brush, a diameter D (m) of the grinding brush, and a running speed V (m/min) of the steel sheet satisfy the following formula (5),
the heat treatment step (d) further provided with
a step (d-1) of heating the steel sheet obtained at the cold rolling step (c) from 650°C to a maximum heating temperature of Ac1+50°C or more and 950°C or less by an average heating speed of 0.5 to 500°C/s,
a step (d-2) of holding the steel sheet obtained at the cold rolling step (c) at the maximum heating temperature for 1 second to 300 seconds,
a step (d-3) of cooling the steel sheet obtained at the cold rolling step (c) down to Ms point-100°C or less in temperature, at which step, cooling from 700°C to 500°C by a 10°C/s or more average cooling speed, and
a step (d-4) of holding the steel sheet obtained at the cold rolling step (c) at 200 to 350°C for 1 to 600 seconds,
at step (d-1), an atmosphere in surroundings of the steel sheet obtained at the cold rolling step (c) having a steam partial pressure pH₂O and hydrogen partial pressure pH₂ satisfying a following formula (6): $\begin{matrix}\frac{R ⋅ D}{V} > 10 \left(5\right) \\ - 1.0 \leq log \left({pH}_{2}O/{pH}_{2}\right) \leq 0.1 \left(6\right)\end{matrix}$

4. The method of production of steel sheet according to claim 3, wherein
the hot rolling step (a) further comprises a step of retaining a heat of the hot rolled steel sheet after coiling within 30 minutes in a heat insulating vessel with inside walls covered by a heat insulating material, wherein
a peak temperature of an atmospheric temperature inside of the heat insulating vessel is 500 to 650°C, and a time from the atmospheric temperature to the peak temperature is 1 to 8 hours.
